

1

2,990,231

PROCESS OF MODIFYING POLYETHYLENE GLYCOL TEREPHTHALATE FABRICS WITH GUANIDINE OR GUANIDINE CARBONATE AND OPTIONALLY THIODIGLYCOL OR O-PHENYL PHENOL

Joseph Nüsslein, Frankfurt am Main, and Carl Kuch, Hofheim (Taunus), Germany, assignors to Farbwerke Hoechst Aktiengesellschaft vormals Meister Lucius & Brüning, Frankfurt am Main, Hochst, Germany, a company of Germany

No Drawing. Filed July 19, 1956, Ser. No. 598,741

Claims priority, application Germany July 25, 1955

13 Claims. (Cl. 8—114.6)

The present invention relates to a process of altering the appearance of fabrics wholly or partially made of polyester fibres.

It is already known that, by means of chemicals, patterns can be produced on a uniform ground fabric which is, for instance, made of acetate fibres or cellulose fibres. Especially in the case of fabrics consisting of fibre mixtures the one fibre may be strongly attacked or even decomposed whilst the other is completely preserved. A classic example in this direction is the so-called burnout article the cellulose fibres of which are destroyed by means of carbonizing agents.

Now we have found that the appearance of fabrics wholly or partially made of polyester fibres can be altered in such a way that they are printed with pastes containing a thickening agent and guanidine or compounds yielding guanidine and that the printed fabric is subjected to a steaming process or to the action of high temperatures. The guanidine is advantageously applied in the form of the carbonate.

By polyester fibres are understood such fibres as are formed from bivalent acids and polyhydric alcohols and contain 6-member carbocyclic rings. There are particularly mentioned the high molecular polyesters on the basis of aromatic dicarboxylic acids, such as terephthalic acid and bihydric aliphatic alcohols such as ethylene glycol, propylene glycol, butylene glycol, dimethyl-propylene glycol.

As thickening agent there may be used the usual printing thickenings such as British gum, crystal gum, tragacanth, polyvinyl alcohol, starch and cellulose derivatives, locust bean flour thickening and the like.

The intensity of the action can be varied according to the time and intensity of the heating or steaming process. The printed parts of the fabric, for example, can become transparent by subsequent steaming. If, however, the fabric is heated to high temperatures, for example to 180° C.—220° C., the printed parts of the polyester fabric are destroyed.

The concentration of guanidine or guanidine carbonate normally ranges between 15 and 45 percent, calculated upon the total quantity of the paste to be applied. By the additional use of auxiliaries intensifying the effect such as thiodiglycol or ortho-phenyl-phenol it is possible to reduce the concentration of guanidine or guanidine carbonate to 5–10 percent. The quantities of the auxiliary should advantageously be within the same range, i.e. between 5–10 percent.

The time of steaming and of the subsequent heating to high temperatures depends on various factors, such as the desired effect, the temperature, the auxiliaries etc. Normally, it suffices to steam for about 30 minutes or to heat for about ½–1 minute, preferably at a temperature ranging between 170° C. and 220° C.

Such printing thickenings having a decomposing effect can be printed on undyed and dyed material, on textiles made solely of polyester fibres and also on such textiles

2

consisting of mixtures of polyester fibres and other fibrous materials, for example, native cellulose, fibres of regenerated cellulose, wool and synthetic fibres such as are made, for example of polyacrylonitrile, superpolyamides and the like.

To the pastes containing the thickening agents and guanidine, advantageously in the form of the carbonate, there may be added other substances, for example dye-stuffs such as dispersion dyestuffs, vat dyestuffs, pigment dyestuffs etc., whereby especially attractive effects can be obtained, particularly in the case of mixed fabrics. Discharging agents may also be used thus yielding further possibilities of variation, for example, by white or coloured discharging.

The following examples serve to illustrate the invention, but they are not intended to limit it thereto, the parts being by weight:

Example 1

60 parts of a mixture consisting of British gum (1:1) and crystal gum (1:2) are mixed with 20 parts of water and 20 parts of guanidine carbonate.

A fabric made of polyethylene glycol terephthalate fibres is printed with the paste thus obtained, dried, heated for 30 seconds to 200° C., rinsed, soaped at the boil, rinsed and dried.

The unprinted parts of the fabric show a dull milky appearance whilst the printed pattern is transparent.

Example 2

50 parts of British gum (1:1) are mixed with 25 parts of guanidine carbonate and 25 parts of water. A fabric made of polyester fibres is printed with the paste thus obtained, dried, heated for 1 minute to 200° C., rinsed, soaped at the boil, rinsed and dried.

The printed parts of the fabric are completely destroyed.

Example 3

A nettle-like fabric made of spun polyester fibre yarn is overprinted, by means of a fine blotch-roller, with a paste consisting of:

50 parts of British gum (1:1), 25 parts of guanidine carbonate, and 25 parts of water.

The fabric is then dried, heated for 1 minute to 200° C., rinsed, dried once more and roughened. Whilst, in view of the high strength of the polyester fibre, the untreated fabric can only be roughened very difficultly, the treated material can be roughened very well. By the choice of appropriate patterns any desired roughening effects can be obtained in such a manner that the printed parts show a denser fleece while the unprinted parts are raised very little. In this manner, even continuous fibres can be advantageously worked up into raised articles.

Example 4

50 parts of British gum (1:1) are mixed with 10 parts of guanidine carbonate, 30 parts of water and 10 parts of thiodiglycol.

A fabric made of polyester fibres is printed with the paste thus obtained, dried, heated for 1 minute to 180° C., rinsed, soaped at the boil, rinsed and dried. The printed parts of the polyester fabric are destroyed.

Example 5

60 parts of British gum (1:1) are mixed with 10 parts of guanidine carbonate, 10 parts of ortho-phenyl-phenol and 20 parts of water. A fabric made of polyethylene glycol terephthalate is printed with this paste, dried, heated for 40 seconds to 200° C., rinsed, soaped at the boil, rinsed and dried.

The printed parts of the fabric are completely removed.  
We claim:

1. A process which comprises printing in selected areas fabrics comprising fibers consisting essentially of polyethylene glycol terephthalate with a printing paste selected from the group consisting of

(1) a paste comprising an inert thickening agent and from about 15 percent to about 45 percent by weight of a member of the group consisting of guanidine and guanidine carbonate,

(2) a paste comprising an inert thickening agent and from about 5 percent to about 10 percent by weight each of thiodiglycol and a member of the group consisting of guanidine and guanidine carbonate, and

(3) a paste comprising an inert thickening agent and from about 5 percent to about 10 percent by weight each of o-phenylphenol and a member of the group consisting of guanidine and guanidine carbonate, all said percentages being based on the total weight of the printing pastes, and then heating the printed fabric at a temperature from about 100° to about 220° C. until complete destruction of the polyethylene glycol terephthalate fibers in the printed area occurs.

2. A process which comprises printing in selected areas fabrics comprising fibers consisting essentially of polyethylene glycol terephthalate with a printing paste comprising an inert thickening agent and from about 15 percent to about 45 percent, based on the total weight of printing paste, of a member of the group consisting of guanidine and guanidine carbonate, and then heating the printed fabric at a temperature from about 100° C. to about 220° C. until complete destruction of the polyethylene glycol terephthalate fibers in the printed areas occurs.

3. A process as in claim 2 wherein said printing paste contains guanidine carbonate.

4. A process as in claim 3 wherein the printed fabric is heated at a temperature from about 170° to about 220° C.

5. A process as in claim 4 wherein said inert thickening agent is British gum.

6. A process which comprises printing in selected areas fabrics consisting essentially of polyethylene glycol terephthalate fibers with a printing paste comprising an inert thickening agent and from about 15 percent to about 45 percent, based on the total weight of printing paste, of a member of the group consisting of guanidine and guanidine carbonate, and then heating the printed fabric at a temperature from about 100° C. to about 220°

C. until complete destruction of the polyethylene glycol terephthalate fibers in the printed areas occurs.

7. A process as in claim 6 wherein said printing paste contains guanidine carbonate.

8. A process as in claim 7 wherein the printed fabric is heated at a temperature from about 170° to about 220° C.

9. A process as in claim 8 wherein said inert thickening agent is British gum.

10. A process which comprises printing in selected areas fabrics comprising fibers consisting essentially of polyethylene glycol terephthalate with a printing paste containing an inert thickening agent and from about 5 percent to about 10 percent by weight each of guanidine

15 carbonates and a member of the group consisting of thiodiglycol and o-phenylphenol, based on the total weight of the printing paste, and then heating the printed fabric at a temperature from about 100° C. to about 220° C. until complete destruction of the polyethylene glycol

20 terephthalate fibers in the printed areas takes place.

11. A process as in claim 10 wherein said temperature is between about 170° to about 220° C.

12. A process which comprises printing in selected areas fabrics consisting essentially of polyethylene glycol 25 terephthalate with a printing paste containing an inert thickening agent and from about 5 percent to about 10 percent by weight each of guanidine carbonate and a member of the group consisting of thiodiglycol and o-phenylphenol, based on the total weight of the printing 30 paste, and then heating the printed fabric at a temperature from about 100° C. to about 220° C. until complete destruction of the polyethylene glycol terephthalate fibers in the printed areas takes place.

13. A process as in claim 12 wherein said temperature 35 is between about 170° to about 220° C.

#### References Cited in the file of this patent

#### UNITED STATES PATENTS

|    |           |         |               |
|----|-----------|---------|---------------|
| 40 | 1,588,951 | Dreyfus | June 15, 1926 |
|    | 2,287,696 | Willer  | June 23, 1942 |
|    | 2,607,655 | Weiss   | Aug. 19, 1952 |
|    | 2,607,656 | Ridge   | Aug. 19, 1952 |

#### FOREIGN PATENTS

|    |         |               |               |
|----|---------|---------------|---------------|
| 45 | 664,921 | Great Britain | Jan. 16, 1952 |
|----|---------|---------------|---------------|

#### OTHER REFERENCES

American Dyestuff Reporter, Nov. 13, 1950, p. 790,  
"The Dyeing Properties of Terylene."